

July 15, 1952

J. C. ECKEL

2,603,577

HIGH-TEMPERATURE BOX ANNEALING PROCESS FOR  
FERROUS VITREOUS ENAMELING SHEET STOCK

Filed Jan. 12, 1949

2 SHEETS—SHEET 1

*Fig. 1.*



*Fig. 2.*



*Fig. 5.*



*Fig. 6.*



*Fig. 7.*



*Fig. 8.*



INVENTOR

JOSEPH C. ECKEL

by Hooper, Leonard & Glenn  
his attorney.

July 15, 1952

J. C. ECKEL

2,603,577

HIGH-TEMPERATURE BOX ANNEALING PROCESS FOR  
FERROUS VITREOUS ENAMELING SHEET STOCK

Filed Jan. 12, 1949

2 SHEETS—SHEET 2

**Fig. 3.**



**Fig. 4.**



**Fig. 9.**



INVENTOR  
JOSEPH C. ECKEL  
by Hooper, Leonard & Clem  
his attorneys

## UNITED STATES PATENT OFFICE

2,603,577

HIGH-TEMPERATURE BOX ANNEALING  
PROCESS FOR FERROUS VITREOUS  
ENAMELING SHEET STOCKJoseph C. Eckel, Pittsburgh, Pa., assignor to  
United States Steel Company, a corporation of  
New Jersey

Application January 12, 1949, Serial No. 70,514

4 Claims. (Cl. 148—12)

1

This invention relates to the quicker, cheaper and more efficient quantity production of iron or steel sheet stock suitable for vitreous enameling. More particularly, it involves the novel application of but a single and unconventional box annealing operation on such enameling sheet stock in loosely coiled strip form at temperatures within the critical range of temperature for such stock.

It is common in vitreous enameling practice to use as the enameling sheet stock a single carbon steel or so-called low metalloid enameling iron or steel having a very low carbon content, usually not in excess of from 0.4% to 0.05% carbon. In one particular practice, the chemical composition of a representative rimmed or open steel used for this purpose might contain, by way of illustration and not limitation to the recited specific proportions: carbon—.03%; manganese—.10%; phosphorus—.015%; sulphur—.030%; silicon—.010%; residual amounts of copper, nitrogen and chromium; with the balance being substantially all iron.

Such steel is frequently made by rolling it into slab form, then hot-rolling the slab on a continuous hot strip mill, pickling the strip to clean and descale it, and cold reducing the strip on a continuous or reversing cold reduction mill to the ordered thickness, if the ordered thickness were below that conveniently attainable by hot-working. The material may or may not be cleaned prior to heat-treating. In one manufacturing process, the steel was then sheared to length and normalized at about 1700° F. sheet temperature, and cooled to about 1000° F. before being air-cooled substantially to atmospheric temperature and pickled. Such sheets had good vitreous enameling characteristics but if additional deep-drawing properties were required, they were then box annealed in the range around from about 1100° F. to about 1250° F. to improve their ductility by relieving any residual stresses resulting from the normalizing treatment. And in some cases, the conventional box annealing step preceded the normalizing.

Normalizing operations by virtue of the larger investment and greater handling add materially to the cost of producing vitreous enameling sheets. Thus, a single or a very limited number of sheets can be treated at one time in normalizing so that the output tonnage per hour of sheets is tremendously curtailed and the unit cost thereof correspondingly increased. Moreover, the air-cooling of the normalized sheets scales them, necessitating subsequent additional handling and ex-

2

pense for further pickling treatment. In addition, the relatively quick cooling achieved by air-cooling adversely affects the softness of the sheets, requiring for some applications the further box annealing step which has been mentioned. Although the cooling of a conventional normalizing operation is faster than the cooling of a conventional box annealing operation, this difference in time is insufficient to make up for the lower tonnage capacity of the usual normalizing operation.

Vitreous enameling sheets are also made from coiled strip of such simple carbon steels in which no normalizing but simply a conventional box annealing step is employed. In such box annealing in one commercial practice the strip is loosely coiled to prevent any sticking or welding tendency and heated in an annealing box to a temperature which is not permitted to exceed a maximum sheet temperature of about 1260° F. Since such box annealing is usually conducted in a neutral or a deoxidizing atmosphere, such as a natural gas atmosphere, no subsequent pickling or other cleaning is usually required or is necessary. For special applications, an oxide coating is sometimes produced by the use of a controlled oxidizing atmosphere during annealing. Moreover, the tonnage output per hour for box annealing is large by comparison with normalizing by reason of the greater weight of metal that can be treated in a conventional box annealing operation in a given time.

However, such subcritical temperature box annealed sheets do not exhibit as a general rule a grain structure characteristic suitable for deep-drawing purposes and hence are confined in their application to limited uses such as simple table tops and other relatively flat panel applications. This is so whether the sheets are sold in cut lengths or in coiled strip form, with or without temper rolling, and even though the usual slow cooling is employed. Nor are the mechanical properties of such sheets so box annealed as good as those of sheets subjected to normalizing alone or to both normalizing and box annealing.

Heretofore in the art of box annealing ferrous vitreous enameling sheet stock, the temperature of such annealing in the enameling sheet art has been carefully kept below the critical range. One reason for this practice was that it had been considered that increasing the temperature of such box annealing favored an objectionable nonuniform grain structure which, if not restricted, upon drawing resulted in the material pulling coarse. When noticeable to the naked eye, it is

known as the "orange peel" effect and destroys the commercial value of deeply drawn sheets intended for finished smooth surface applications. Moreover, when sheets instead of loosely coiled strip are box annealed above about 1300° F. the sticking or welding tendency of the sheets increases to an extent which makes such box annealing of stacked sheets impracticable if tonnage production and acceptable product yield are to be maintained. If such sticking occurs, the sheets or strip may have to be rejected or they may tear in subsequent handing.

Box annealing in such subcritical temperature ranges as a rule does not effect complete recrystallization of the grain structure of the sheet or strip. However, it did stress relieve the grain structure by producing sufficient reformation thereof to provide suitable softness and ductility in the finished sheet or strip for very limited applications. Such conventional box annealing below the critical temperature also relieved strains produced by prior cold-working or any prior normalizing of the metal.

Aside from the normal metallurgical reasons, there was another and possibly more substantial one in the vitreous enameling sheet stock art for maintaining the maximum sheet temperature at about 1260° F. in the box annealing operation. It had been determined that unstable carbon or carbide formations resulted at higher box annealing temperatures which moved into the critical temperature range. Without the following belief being intended to limit the scope of this invention in any way, it appears that such carbides tend to agglomerate and form unstable "rosettes" in the sheets or strips when box annealed from between about 1260° F. to 1300° F. as a lower limit and about 1450° F. as an upper limit. Subsequently, upon the firing of a vitreous enamel coat on such sheets at temperatures approximating about 1550° F., mirror design blisters or "curtains" or copperheads overlying such "rosettes" too frequently result in the enamel product and cause its rejection. These rosettes appear to be large pearlitic patches of unstable character which combine with the oxides in the vitreous enamel frit and give off gases. As a consequence, the industry has never applied box annealing to vitreous enameling iron sheets or strips at sheet temperatures above substantially about 1260° F. Nor has it considered such a box annealing operation suitable for producing sheets with good drawing properties without combining it with a further annealing or normalizing operation.

The present invention for the first time provides a process in which a single unconventional box annealing operation is employed for making vitreous enameling sheets or strips having good firing, drawing and mechanical characteristics and properties. In addition, the grain structure produced by the practice of this invention not only has good drawing properties but it is substantially uniform in character. This invention eliminates the need for normalizing or for combining of a normalizing and conventional box annealing in the commercial production of such enamel sheet stock. The carbon or carbides in the sheets produced in accordance with this invention are either so dispersed or so stabilized as to eliminate previous rejections because of such blisters and copperheads. Hence, the cost of producing suitable ferrous enameling sheets is hereby markedly reduced and the art materially advanced. Other objects and advantages of this

invention will appear from the drawings, which are illustrative only, in which

Figure 1 is a vertical cross section through a gas-fired radiant tube annealing box;

Figure 2 is a section taken along line II-II of Figure 1;

Figure 3 is a diagram showing typical annealing temperatures in conventional sheet or coil box annealing for enameling sheet stock;

Figure 4 is a diagram showing a typical conventional normalizing curve for enameling sheet stock;

Figure 5 is a diagrammatic view of a portion of the iron-carbon phase diagram illustrating the temperature ranges employed in prior ferrous enameling sheet production practices;

Figure 6 is a diagrammatic view of a portion of the iron-carbon phase diagram illustrating the critical temperature range employed in this invention;

Figure 7 is an enlarged representative pictorial view of unstable "rosettes," etched to bring out the carbide structure and grain boundaries;

Figure 8 is an enlarged representative pictorial view of the material shown in Figure 7 etched to bring out the carbide structure only and not the grain boundaries; and

Figure 9 is an enlarged representative pictorial view of a section of a sheet made in accordance with this invention in which the carbides are in substantially stable and dispersed form, said sheet being etched to bring out the carbon elements only.

Referring to Figures 1 and 2, a common practice in conventional box annealing involves the use, in one type of annealing furnace, of a so-called radiant tube annealing box. Such a box comprises a heavy cast metal base 10 usually covered by a low platform of refractory brick 11 which platform ends short of the outer edge of base 10. A radiant tube annealing box 12 of metal lined with refractory brick 13 and having an arched refractory top portion 14 is supported by base 10 when closed and fits over platform 11 during the annealing operation. The annealing charge may or may not be covered by a retort or inner cover. Between operations, box 12 is lifted out of the way by a crane engaging eyes in ears 12' on box 12. Heat is supplied to the interior of the annealing box by banks of radiant tubes 15 within which natural gas or other suitable fuel is burned causing the tubes to become incandescent. A deoxidizing atmosphere, such as natural gas, is preferably recirculated through the interior of box 12 by means of pipe connections 16, and maintained at a pressure slightly greater than atmospheric so that air will not have access to the said interior thereof. And sometimes no outside gas is circulated through the annealing box. A gas seal is provided when box 12 is closed by a sand or powdered refractory ring 17 around the base of box 12. In the described practice, loosely coiled material 17 of hot or cold reduced ferrous enameling strip stand on edge singly or in stacks on platform 11 to prevent sticking.

In the prior practice, such coils are heated to a so-called maximum sheet temperature of about 1250° F. In so doing, allowance has to be made for the temperature differential of possibly 75° F. or higher between the top outer edges and bottom centers of the sheet or coils, a differential which exists in all box annealing furnaces as illustrated in Figure 3. As mentioned earlier, the stacking of sheets imposes temperature limi-

tations due to the tendency to stick which are not present when loosely coiled strips are box annealed in accordance with the preferred conventional practice in the art. In some cases, the sheets can be stacked vertically and spaced to avoid sticking but such a method is not practical by comparison with annealing loose coils. However, even when conventionally annealing loose coils or spaced sheets the problem of the poor grain structure for drawing remains. As shown in Figure 3, such coils are generally held at annealing temperature for from about 10 to 20 hours to insure obtaining as much of the softness and ductility required and appropriate grain as possible in the finished sheet. Such sheets whether sold in cut lengths or in the form of coiled strip, had good enameling properties but poor drawing and mechanical properties as mentioned earlier.

On the other hand, when such sheets are subjected, as illustrated in Figure 4, to the more costly normalizing in the temperature range extending upward from the  $A_3$  point which for steel compositions of the type with which this invention deals varies upwardly from about  $1625^{\circ}$  F. for a period of time at temperature varying from about 1 to 4 minutes, the entire grain structure is recrystallized and made uniform. Such a normalized product also has good enameling properties, and a somewhat improved drawing property insofar as grain structure is concerned. However, the relatively rapid air-cooling to which normalized sheets are subjected has a hardening effect and imparts strains which require further box annealing if extra deep-drawing qualities are to be obtained.

Such prior conventional practice with respect to box annealing and normalizing either separately or in combination in the production of ferrous enameling sheet stock is depicted in Figure 5 in which a shaded line 18 diagrammatically illustrates the lower critical temperature limit or the  $A_1$  line and an upper shaded line 19 represents the upper critical or  $A_3$  limit. A shaded line 18a indicates that part of the conventional line of phase change in the iron-carbon diagram extending from line 18 at about 0.035% carbon substantially to the  $A_3$  line 19. The shading is employed in order to portray in an approximate manner the spread applicable in the precise location of these critical limits for metals of different composition and for the respective heating and cooling operations in that range for a given steel. The intermediate  $A_2$  limit where the alpha iron changes to the beta form is illustrated by a line 20. The prior practice in box annealing in ferrous enameling stocks confined such annealing substantially to the crosshatched zone marked 21, while normalizing of such enameling sheet stocks took place in the crosshatched zone marked 22. But operations within the critical range between the  $A_1$  and  $A_3$  limits for a given composition of ferrous enameling sheet or strip have heretofore been considered deleterious and impossible for any satisfactory result.

The present invention is depicted diagrammatically in the phase diagram of Figure 6 in which the line of phase change, corresponding to line 18a in Figure 5, is indicated at 23 and the  $A_3$  limit at 24 with the  $A_2$  line being designated by the numeral 25. A vertical line 26 represents a typical composition ferrous enameling sheet or strip steel containing about 0.025% carbon. Under this invention, the box annealing of such strip in loosely coiled form in a suitable box an-

nealing furnace such as that illustrated in Figures 1 and 2 is carried on at a temperature within the critical temperature range of such steel for a period of time at temperature, commonly called the soaking period, necessary to obtain a suitable, soft, ductile quality and substantially uniform grain structure, before cooling is permitted to begin. Such box annealing between line 23 or the  $A_1$  line and the  $A_3$  points not only produces a sheet having good deep-drawing and mechanical properties but it also conditions the carbide formation and renders it sufficiently stable so that in the subsequent vitreous enameling firing operation mirror design blisters and copperheads do not occur to any commercially detrimental extent. Carbon rosettes, including grain size, are illustrated in Figure 7 at an approximate magnification of 1000 times, using an etchant called nital (ethyl or methyl alcohol and nitric acid) to bring out the thin dark lines which are the grain boundaries and the large black areas which are the pearlitic patches called "rosettes." Such rosettes as may be formed by the agglomeration of the carbon or carbide elements in the enameling sheet stock by raising the temperature above the lower critical or  $A_1$  limit, when etched specifically for carbides with sodium picrate and at the same approximate magnification have the general appearance illustrated in Figure 8. When, however, ferrous vitreous enameling sheet stock is processed in accordance with this invention, such carbides are relatively dispersed and are stabilized and take the form as depicted by the illustration in Figure 9, using an etchant such as sodium picrate at approximately the same magnification. The carbide structure of Figure 9 does not give rise to the gas evolution difficulties in the vitreous enamel firing step which are occasioned when the carbides are in the form shown in Figures 7 and 8.

Some latitude is permissible in the time and temperature relationship which in a given case employing the instant invention would permit of some change in time element for a corresponding and inverse change in temperature element. By way of illustration of the time-temperature relationship, sheets treated in accordance with this invention exhibited a Rockwell "B" hardness between 38.5 and 39.0 with a grain size number of 6 to 7 when the respective sheets were treated at  $1500^{\circ}$  F. for 4 hours; at  $1550^{\circ}$  F. for 2 hours and at  $1625^{\circ}$  F. for 1 hour. In one suitable so-called austenitic grain-size chart commonly used for the classification of grains, the following numbers are given to the designated range of grain sizes measured in grains per square inch at 100 magnifications:

| 60 | Grain Size No. | No. of Grains per Sq. In. at 100 X |
|----|----------------|------------------------------------|
| 3  |                | 1½-6                               |
| 4  |                | 6-12                               |
| 5  |                | 12-24                              |
| 6  |                | 24-48                              |
| 7  |                | 48-96                              |
| 8  |                | 96-125                             |

Similarly, some latitude exists in the heat input rates, the cooling rates, and the components of the stock as to which in order to obtain one or more special effects some other factor or factors may be slightly compromised without departing from the scope of this invention.

Further, the practice of this invention yields a ferrous enameling sheet in which the grain struc-

ture is of a grain size number varying from about 5 to 8 and substantially uniform, thereby insuring the drawability and uniformity of the new sheet. This would not be the situation if in the box annealing the top sheets which are hotter by the amount of the temperature differential in the annealing furnace between the bottom and top sheets, are permitted to exceed the  $A_3$  temperature limit for any prolonged period of time because then the grain structure in those top sheets would tend to grow to objectionable size for drawing (grain size numbers up to about 4) and might instead of being uniform be a combination of very large size surface grains and relatively small size grains at the center of the gage.

In the preferred practice of this invention, such box annealing of a typical simple carbon steel enameling stock takes place within the temperature range from about  $1500^{\circ}$  F. to about  $1600^{\circ}$  F. with a suitable soaking time and slow conventional cooling. This soaking time may vary from the order of from about 2 to about 10 hours and is a material reduction in time over prior practice and hence materially boosts capacity achieved under this invention on still another count. The charge in the furnace might be brought up to annealing temperature within about 30 to 40 hours, soak and be cooled out of the air and under cover to about  $300^{\circ}$  F. (usually at a rate not in excess of a maximum of  $200^{\circ}$  F. per hour) before being cooled in the open the rest of the way down to atmospheric temperature. Where very fine temperature control can be obtained, the hottest portion of the sheets or strip being so box annealed should be maintained as much on the high side in the critical range and just below the  $A_3$  point as possible for a given composition. In general, it has been observed that by means of a single box annealing operation ferrous vitreous enameling sheets treated in accordance with this invention may be obtained with a Rockwell "B" hardness between 33 and 38 approximately, with yield points varying between 21,000 and 26,000 pounds per square inch approximately, with an ultimate strength varying between 40,000 and 42,800 pounds per square inch approximately, with a percentage elongation in 2" varying between 36.5 and 41 approximately; and with a grain size about 5 to 6 approximately, when annealed at about  $1600^{\circ}$  F. for about 4 hours. These figures are but an indication of the highly useful and unexpectedly satisfactory results which are obtainable by the practice of this invention.

In the following representative comparison ferrous enameling sheet stock typical of the type considered herein will under one practice of this invention and under conventional normalizing give the following estimated results, although this invention is not to be limited to the specific figures shown:

|                                                 | Annealing by Present Invention Between $A_1$ and $A_3$ Points | Conventional Normalizing Above $A_3$ Point |
|-------------------------------------------------|---------------------------------------------------------------|--------------------------------------------|
| Bottom temperature (of material), $^{\circ}$ F. | 1,525                                                         | 1,700                                      |
| Top temperature (of material), $^{\circ}$ F.    | 1,600                                                         | 1,700                                      |
| Time to bring to temperature                    | 30 hours                                                      | 4 minutes                                  |
| Soaking period                                  | 3 hours                                                       | 2 minutes                                  |
| Cooling time before reaching air                | 12 hours                                                      | 12 minutes                                 |
| Yield point, lbs./in. <sup>2</sup>              | 21,800-28,400                                                 | 26,000-32,000                              |
| Ultimate strength, lbs./in. <sup>2</sup>        | 40,000-43,000                                                 | 44,000-46,000                              |
| Per cent. Elongation in 2"                      | 36-40                                                         | 33-37                                      |
| Olsen Ductility                                 | .360-.430                                                     | .370-.420                                  |
| Rockwell "B" Hardness                           | 33-38                                                         | 40-47                                      |
| Grain Size No.                                  | 5-6                                                           | 5-6                                        |

It will be noted the grain size obtained in the practice of this invention is uniform and substantially no larger than the grains produced by normalizing. Although the annealed steel has a yield point which is somewhat lower than the normalized product, any such lowering offers a greater spread in the plastic range before failure and therefore contributes to the drawing qualities of the metal. Furthermore, the slow cooling of the box annealing in accordance with this invention avoids the hardening and strain risks attendant upon the use of the more expensive conventional normalizing without objectionable grain growth.

15 In one annealing operation of a coil charge of 120 tons in accordance with this invention, it required 41 hours for the charge to reach a metal temperature of  $1575^{\circ}$  F.- $1625^{\circ}$  F., at which temperature the charge was held for a period of about 4 hours. The gage of the metal in the coils varied from .0359 to .0478". After annealing, the grain size numbers of the charge ranged from 5 to 7; the Rockwell "B" hardness ranged between 31 and 41 and averaged 37; the yield 20 strength of the charge in pounds per square inch ranged from 21,000 to 28,100; the ultimate strength from 40,000 pounds to 45,800 pounds per square inch; and the percentage elongation in 2" ranged from 32 to 41. These results are 25 but one example of the advantages of this invention.

30 Although I have illustrated and described a preferred practice and embodiment of the invention, it will be understood that changes may be made therein without departing from the spirit of the invention or the scope of the appended claims.

I claim:

1. A process for imparting ductility and carbide stability to very low carbon ferrous vitreous enameling sheet stock after completion of the reduction thereof to an ordered thickness, comprising box annealing said sheet stock in loosely coiled strip form between about  $1500^{\circ}$  F. and about  $1600^{\circ}$  F. for a period of time sufficient substantially to stabilize the carbides therein, and then relatively slowly cooling said stock.

2. A process for producing a finally annealed low metalloid ferrous vitreous enameling sheet stock, comprising cold reducing a strip of enameling steel to an ordered thickness of said stock, releasing the coiling tension of said cold reduced stock, loosely recoiling said stock, arranging said loosely coiled strip in a box annealing furnace on edge, annealing said loosely coiled stock in said furnace between about  $1500^{\circ}$  F. and about  $1600^{\circ}$  F. for a soaking period of time sufficient to stabilize the carbides and varying between about 2 hours and about 10 hours, slowly cooling said 45 annealed stock substantially to atmospheric temperature, and maintaining a nonscaling atmosphere about said loosely coiled stock during said annealing and said slow cooling until said loosely coiled stock has reached a temperature of about 50  $300^{\circ}$  F., whereby commercially practicable vitreous enameling sheets are produced having stable carbides, a maximum Rockwell "B" hardness of 55 40, a minimum percentage elongation in 2" of about 32, a minimum yield point of about 22,000 pounds per square inch, a minimum ultimate strength of about 38,000 pounds per square inch, and a maximum grain size number of about 5.

60 5. In a method of making enameling sheets, the steps including cold-rolling low-carbon ferrous strip suitable for vitreous enameling sub-

stantially to final gauge, coiling the strip leaving the turns of the coils loose, box annealing the resulting coils by heating them in a non-oxidizing atmosphere to a temperature between 1550 and 1650° F., then cooling them in said atmosphere to about 300° F. thereby eliminating the tendency of sheets cut from the strip to exhibit mirror blisters on vitreous enameling.

4. In a method of making enameling sheets, the steps including rolling low-carbon ferrous strip suitable for vitreous enameling substantially to final gauge, coiling the strip leaving the turns of the coils loose, box annealing the resulting coils by heating them in a non-scaling atmosphere to a temperature between about 1550° F. and 1650° F., then cooling them in said atmosphere thereby preparing them for vitreous enameling.

JOSEPH C. ECKEL.

#### REFERENCES CITED

The following references are of record in the file of this patent:

#### UNITED STATES PATENTS

| Number       | Name       | Date         |
|--------------|------------|--------------|
| 1,536,663    | Cunningham | May 5, 1925  |
| 1,723,152    | Grafton    | Aug. 9, 1929 |
| 10 1,887,215 | Ruder      | May 10, 1932 |
| 1,996,568    | Butts      | Apr. 2, 1935 |

#### OTHER REFERENCES

"Metals Handbook," 1948 ed., p. 354, published by American Society for Metals.

15 "The Metallurgy of Deep Drawing and Pressing," by Jevons, pp. 199-200, John Wiley & Son, 1942.